

# UNITED STATES PATENT OFFICE.

ALBERT STRASSER, OF RORSCHACH, SWITZERLAND.

## PROCESS FOR DEOXIDIZING ALUMINUM AND ITS ALLOYS.

1,848,458.

specification of Letters Patent.

Patented Aug. 3, 1920.

No Drawing.

Application filed February 5, 1920. Serial No. 356,547.

To all whom it may concern:

Be it known that I, ALBERT STRASSER, a citizen of Switzerland, residing at Rorschach, Canton of St. Gall, Switzerland, 5 have invented certain new and useful Improvements in Processes for Deoxidizing Aluminium and Its Alloys, of which the following is a specification.

This invention has for its object to provide an improved process for deoxidizing aluminium and its alloys which consists in adding to the aluminium heated above its melting point, first an aluminium cartridge containing potassium phosphid ("kalium phosphoricum") for the purpose of converting the impurities (consisting of Si, and Fe, and also O) into phosphorus compounds; and then, when the aluminium has reached a still higher temperature, adding 10 a second aluminium cartridge charged with one of the metals of the alkaline earths, for the purpose of oxidizing the phosphorus compounds, the resulting reaction being such that the phosphorus compounds burn 15 at the expense of the alkaline earth metal used, and the oxids form slag which floats on top of the aluminium, being insoluble in aluminium.

### Example.

30 The aluminium is heated to a temperature above its melting point, for instance to 800 degrees centigrade. Then an aluminium cartridge filled with potassium phosphid ("kalium phosphoricum") is added to the bath of molten metal. Since the cartridge has a higher specific gravity than the liquid aluminium, the cartridge sinks to the bottom of the crucible and is melted there. 35 The potassium phosphid becoming thereby released, diffuses throughout the bath of molten metal, and the impurities are converted by the phosphorus entering into reaction, into phosphor metals without affecting the aluminium, because the affinity of the phosphorus to aluminium is not so great as to the aforesaid metals Si and Fe.

The temperature of the aluminium is now raised to about 1100 degrees C., whereupon 40 the second cartridge filled with one of the metals of the alkaline earths, such as for instance, calcium, barium, strontium, lithium, etc., is added to the bath of molten metal. The alkaline earth metal combines 45 (with generation of heat) with the oxygen present as an impurity in the aluminium,

and also with the phosphids of Si and Fe, while the oxids of the metals Si and Fe, and the oxygen compounds of the aluminium rise, together with the respective metallic 60 oxid, to the surface of the metal bath and are no longer soluble in the latter.

This deoxidation of aluminium produces a finer structure and a higher density of the metal.

As a consequence of mechanical treatment of the deoxidized metal its tensile strength is thrice that of the metal before deoxidation.

Its electric resistivity is diminished, 70 whereas its conductivity is increased, which is an important advantage especially in the case of electric line wires.

The additions are used only in quantities up to 1.5 per cent., so that the whole of the 75 metal is consumed in the reaction, and none of the alkaline earth metal remains in solution in the aluminium.

### What I claim is:

1. A process for deoxidizing aluminium 80 and its alloys, which consists in first adding an aluminium cartridge containing a phosphorus compound to the aluminium heated above its melting point, for the purpose of converting the impurities into phosphorus 85 compounds, and then when the aluminium has reached a higher temperature, adding a second aluminium cartridge filled with one of the metals of the alkaline earths, for the purpose of oxidizing the phosphorus 90 compounds, the reaction being such that the phosphorus compounds burn at the expense of the alkaline earth metal, and the oxids being insoluble in aluminium, float on the 95 top of the latter.

2. A process for deoxidizing aluminium and its alloys, which consists in first adding an aluminium cartridge containing potassium phosphid ("kalium phosphoricum") to the aluminium heated above its melting 100 point, for the purpose of converting the impurities (consisting of Si, Fe, and O) into phosphorus compounds; and then when the aluminium has reached a higher temperature, adding a second aluminium cartridge 105 filled with one of the metals of the alkaline earths, for the purpose of oxidizing the phosphorus compounds, the reaction being such that the phosphorus compounds burn at the expense of the alkaline earth metal, 110 and the oxids being insoluble in aluminium, float on the top of the latter.

3. A process for deoxidizing aluminium and its alloys, which consists in first adding an aluminium cartridge containing potassium phosphid (kalium phosphoricum) to the aluminium heated to 800 degrees C. for the purpose of converting the impurities (consisting of Si, Fe, and O) into phosphorus compounds, and then when the aluminium has reached a higher temperature, adding a second aluminium cartridge filled with one of the metals of the alkaline earths, for the purpose of oxidizing the phosphorus compounds, the reaction being such that the phosphorus compounds burn at the expense of the alkaline earth metal, and the oxids being insoluble in aluminium, float on the top of the latter.

4. A process for deoxidizing aluminium

and its alloys, which consists in first adding an aluminium cartridge containing potassium phosphid (kalium phosphoricum) to the aluminium heated above its melting point, for the purpose of converting the impurities (consisting of Si, Fe, and O) into phosphorus compounds, and then when the aluminium has reached a higher temperature, adding a second aluminium cartridge filled with calcium for the purpose of oxidizing the phosphorus compounds, the reaction being such that the phosphorus compounds burn at the expense of the calcium, and the oxids being insoluble in aluminium, float on the top of the latter.

In testimony whereof I have affixed my signature.

ALBERT STRASSER.